

E. A. CUSTER.  
ART OF CASTING HOLLOW STRUCTURES IN PERMANENT MOLDS.  
APPLICATION FILED DEC. 10, 1908.

922,754.

Patented May 25, 1909.

Fig. 1.



Fig. 2.



Fig. 3.



WITNESSES:

Thomas M. Smith,  
G. M. Connerston

INVENTOR  
Edgar A. Custer  
BY  
J. Walter Daylan  
ATTORNEY.

# UNITED STATES PATENT OFFICE.

EDGAR ALAN CUSTER, OF PHILADELPHIA, PENNSYLVANIA, ASSIGNOR TO THE CUSTER  
SANDLESS CASTING COMPANY, A CORPORATION OF DELAWARE.

## ART OF CASTING HOLLOW STRUCTURES IN PERMANENT MOLDS.

No. 922,754.

Specification of Letters Patent.

Patented May 25, 1909.

Application filed December 10, 1908. Serial No. 466,765.

*To all whom it may concern:*

Be it known that I, EDGAR ALAN CUSTER, a citizen of the United States, residing at the city of Philadelphia, in the county of Philadelphia and State of Pennsylvania, have invented certain new and useful Improvements in the Art of Casting Hollow Structures in Permanent Molds Having Permanent Cores, of which the following is a specification.

10 My invention has relation to the art of casting bath-tubs, urinals, bowls and various other hollow structures in a sectional permanent mold, whereof one section thereof forms the permanent core; and in such connection it relates particularly to pouring and chilling molten metal swiftly to the point of setting to form homogeneous hollow metal structures, removing the mold-section and finally the cast homogeneous hollow structure, to permit then, if required, the enameling of the structure, for subsequent use.

15 My invention stated in general terms, consists of the art of producing hollow metal cast homogeneous structures in substantially the manner hereinafter described and claimed.

20 The nature, general scope and characteristic features of my invention will be more fully understood from the following description taken in connection with the accompanying drawings forming part hereof, showing one type of means well adapted for expeditiously carrying into effect the defined mode of my said invention, in which—

25 Figure 1, is a front elevational view, in broken section, of a permanent sectional mold having a permanent sectional core for casting therein a bath-tub or the like. Fig. 2, is a transverse sectional view on the line  $x, x$ , of Fig. 1; and Fig. 3, is a sectional view, in detail of a temporary sand core for use in a permanent sectional mold having a permanent metal core, as part of the same, when castings or structures are to be provided with lugs or projections, the said sand core is so arranged as to be set into the sectional permanent mold for enabling the lugs or projections with the main casting produced to be removed therewith.

30 Referring to the drawings 4, is a vertical permanent metal mold, comprising the hinged sections  $a$  and  $b$ ,  $b$ , provided with pour-holes  $c$ ,  $c$  and  $c'$ , having channel-way branches  $c^2$ ,  $c^3$ , leading directly to a central depression corresponding to substantially the

shape or form of the structure to be cast therein. The mold sections are offset in one part to form when the two sections of the mold are united a receptacle  $c^4$ , to receive sand or other molding material, for use, in instances where the hollow article or structure to be cast is to be provided with lugs or projections and this arrangement enables such a casting so provided with lugs or projections to be freed from the mold, with the main portion of the structure cast and as an integral part thereof. The wall of the part  $b$ , of the mold 4, may be provided, as shown in Fig. 2, with tubular openings for passing a fluid therethrough, for water cooling, the same. In the form of the mold, as clearly shown in Fig. 2, the part or section  $a$ , in the making of bowls, bath-tubs or the like, really is in fact the permanent core of the metal hinged sectional mold and the space  $a^2$ , in rear thereof and conforming to the shape or form of the core section, may be cooled with a fluid, as water. Projecting from the section  $b$ , of the mold are rods  $d$ ,  $d'$ , preferably adapted to be fitted with a detachable clamping-bar  $d^2$ , or other means, as clearly shown in Figs. 1 and 2. The type of the sectional mold, combining a permanent core therewith may be employed either vertically or horizontally and good results obtained, in the casting of different kinds or types of hollow metal structures, for being thereafter enamelled, in some instances, for use.

Having thus described the nature and object of my invention, what I claim as new and desire to secure by Letters Patent is:

1. The art of casting hollow metal structures, which consists in chilling swiftly molten metal to the point of setting within a permanent sectional metal mold in which one section thereof is the core of the mold and then cooling through the freeing of the mold section from the cast structure.

2. The art of casting hollow metal structures, which consists in chilling swiftly molten metal to the point of setting within a permanent sectional mold in which one section is the cooled metal core of the mold, hastening cooling of the structure cast to fix the established homogeneity of the said structure by freeing the mold section from the core-section and finally, removing the cast structure.

3. The art of casting hollow metal structures, which consists in chilling swiftly mol-

ten metal to the point of setting within a permanent sectional mold in which one section is the fluid cooled metal core of the mold, then cooling the cast structure through freezing the mold section and finally removing the said cast structure from the core section of the mold.

In witness whereof, I have hereunto set my signature in the presence of two subscribing witnesses.

EDGAR ALAN CUSTER.

Witnesses:

J. WALTER DOUGLASS,  
THOMAS M. SMITH.